

Jan. 18, 1938.

S. RUBEN

2,105,552

INSULATED WIRE

Filed Sept. 3, 1932



*Samuel Ruben*  
INVENTOR.

BY *Samuel Ruben*  
ATTORNEY.

## UNITED STATES PATENT OFFICE

2,105,552

## INSULATED WIRE

Samuel Ruben, New Rochelle, N. Y., assignor to  
 Vega Manufacturing Corporation, Wilmington,  
 Del., a corporation of Delaware

Application September 3, 1932, Serial No. 631,654

4 Claims. (Cl. 173—264)

This invention relates to insulated wires and to the composition of the insulating material thereof.

An object of the invention is to produce a flexible insulated wire having a metallic covering over the insulation.

Another object is to produce a flexible insulated wire having a non-conductive metallic covering.

10 Further objects will be apparent in the disclosure.

Broadly, it may be stated that the invention consists of a metal conductor, an insulating coating over said conductor and a metallic covering 15 over said insulation.

20 The metallic covering may be applied to practically all of the types of insulated wire, for instance, wire having an enamel type insulation of the spirit varnish, oil-resinous, cellulose, glyptal classes, etc., vitreous enamelled wire; rubber insulated wire; oxide-resin insulated wire; silk, paper, cotton, regenerated sheet cellulose wound or asbestos insulated wire.

25 The metallic covering may be applied in several different ways. A low melting point metal or alloy, such as lead-tin, may be melted and wiped on the insulated wire. Or finely divided low melting point metal or alloy may be mixed with a carrier adapted to burn off under heat and the wire may be passed through this mixture and heated to a point where the metal or alloy melts or flows and the carrier burns out, thus leaving a metallic sheath. Or a finely divided metal having a non-conductive surface, such as flaked 30 or powdered aluminum may be mixed with a resinous or other type carrier, and baked on the insulated wire.

35 A particularly useful metallic coated wire of this type may consist of an insulated conductor 40 of the type described in my copending application: 580,531 of 12th December, 1931, and Patents numbered 1,896,043, 1,896,041 and 1,896,042 issued January 31st, 1933, with a coating of finely divided aluminum and a water insoluble resinous binding material. The insulated wire may be 45 prepared as follows: An oleoresinous varnish consisting of ester and kauri gums, China-wood and linseed oil, turpentine and mineral thinner, is first made up by heating these materials together, in proper proportion, to 500° F. A further compound consisting of one part China-wood oil, one part fish oil and one part phenol-formaldehyde resin is then made up by heating these three materials together at 450° F. for fifteen minutes. Three parts of this latter com-

5 pound are added to seven parts of the ester-kauri gum compound, thus, producing a varnish of good quality for the purposes of this invention. 400 cc. of this varnish are ground with 200 grams of a finely divided refractory material, preferably, an oxide such as iron oxide and after the mixture has been thoroughly ground so that the oxide particles have been reduced to a very fine dimension, the compound is applied to the wire.

10 In some instances it is desirable to add and 45 grind in an inorganic high temperature binder material, such as boric acid, to the insulating compound to obtain adhesion at high temperatures. The use of this borate or inorganic binder is set out in my copending cases heretofore mentioned. Preferably, this inorganic binder should have a melting or fluxing point below the carbonization point of the organic materials used in the coating.

15 In insulating this wire, a continuous coating 20 process is used, the wire passing through cups containing the insulating compound and being heated and baked in ovens located between the cups. If necessary, the compound may be 25 thinned out with suitable solvent thinners such as naphtha, xylol, toluol, etc.

20 The thickness of the coating may be the standard thickness set by the American Engineering Standards Committee for enamel insulated 30 wire or may be less or greater, depending upon the flexibility, dielectric strength, abrasion resistance, etc., required. Likewise, the amount of refractory material, such as the oxide, may be determined by the degree of heat resistance necessary. Generally, it may be stated that the amount of refractory 35 material should be such that after the wire has been wound into coils, it will afford a non-conductive spacer between turns even though the dielectric organic carrier or binder, such as varnish, should become carbonized or burn out. 40

45 In preparing the metallic covering I may use materials in the following proportion: to 400 cc. of the phenol-oil varnish hereinabove described, I add 100 grams of flaked or finely divided aluminum. This aluminum is non-conductive, probably due to the thin film of oxide which seems to naturally form upon the surface and the thickness of this insulating film can be materially increased by chemical treatment, as for instance, by immersion in nitric acid. A thin smooth coat- 50 ing of the aluminum varnish is applied to the wire in a manner similar to the application of the oxide-varnish, the insulated wire passing through cups containing the aluminum varnish compound and being baked on in ovens located between the 55

cups. If desirable an inorganic binder, such as boric acid, may be added to the aluminum varnish.

It will be found that metallic insulated wire 5 of this type is resistant to harmful corona effects and when the metal is properly applied a dense, flexible, abrasion-resistant, water and fire proof coating is had.

To illustrate the invention, reference is made 10 to the drawing.

In the figure the wire (1) has an insulating coating (2) consisting of finely divided iron oxide, held upon the wire by a dielectric resinous binder and has an outer coating (3) consisting of a 15 baked on aluminum varnish mixture. It is understood that the insulating coating (2) might consist of rubber, or an enamel type varnish as described instead of oxide-resin.

The metallic coatings illustrated may be applied to any of the types of insulated wire in use or hereinabove described. In the claims the terms "insulation", "insulated" and "non-conductive" 20 are used in relation to electricity.

I claim:

1. A wire having an inner insulation coating including finely divided iron oxide and having an outer coating comprising finely divided aluminum held on said insulated wire by a water insoluble binder.

2. An insulated wire having an inner insulation coating containing finely divided particles of iron oxide and an outer non-conductive coating over its insulation coating consisting substantially of finely divided aluminum, a binder and a boron 10 compound.

3. A wire having an insulation containing a finely divided refractory oxide material, an organic binder, an inorganic binder compound and having an outer non-conductive coating comprising finely divided aluminum held on said insulated wire by a water-insoluble binder.

4. A wire having an insulation containing a finely divided refractory oxide material, a boron compound, and organic binding material, and 20 a non-conductive coating of finely divided aluminum held on said insulated wire by a water-insoluble binder.

SAMUEL RUBEN.